

May 29, 1951

R. H. K. THOMSON ET AL

2,555,065

METHOD OF TREATING A TOW OF FILAMENTS OR THREADS

Filed Jan. 14, 1948

2 Sheets-Sheet 1

Fig. 1.



Fig. 2.



INVENTORS:

Robin Hamilton Kendall Thomson,  
William Edward Tetlow,  
Archibald Montgomery McDonald,  
BY Cushman, Darby & Cushman  
ATTORNEYS.

May 29, 1951

R. H. K. THOMSON ET AL

2,555,065

METHOD OF TREATING A TOW OF FILAMENTS OR THREADS

Filed Jan. 14, 1948

2 Sheets-Sheet 2

Fig. 3.



Fig. 4.



Fig. 5.



INVENTORS:

Robin Hamilton Kendall Thomson,  
William Edward Tetlow,  
Archibald Montgomery McDonald,  
BY Cushman, Darby & Cushman  
ATTORNEYS.

## UNITED STATES PATENT OFFICE

2,555,065

## METHOD OF TREATING A TOW OF FILAMENTS OR THREADS

Robin H. K. Thomson, Largs, William E. Tetlow, Saltcoats, and Archibald M. McDonald, Kilmarnock, Scotland, assignors to Imperial Chemical Industries Limited, a corporation of Great Britain

Application January 14, 1948, Serial No. 2,246  
In Great Britain March 10, 1947

4 Claims. (Cl. 8—151.2)

1

The present invention relates to a method of treating a tow of filaments or threads in a limited space.

In the manufacture of filaments or threads it frequently happens that the filaments or threads have to be submitted for an appreciable period of time to one or more operations of wet or dry processing. It is desirable to carry out the manufacture of said artificial filaments or threads in as continuous a manner as possible, but as the different operations included in the manufacture may take differing periods of time to complete, some of them appreciable periods, much space and large quantities of reagents may be required if they are to be carried out on a continuously advancing tow of filaments or threads.

The object of the present invention is to provide a simple and efficient method of treating under non-tensioning conditions a continuous travelling tow of filaments or threads by immersion in a treating liquid, particularly one having a specific gravity approaching that of said tow, for relatively long periods of time.

It is known to be impracticable to allow a continuous travelling tow of filaments or threads to fall into and accumulate or form folds in a treating-liquid contained in a static tank of large but reasonable dimensions. The tow becomes entangled if a sufficient length is permitted to accumulate in the tank for it to receive the necessary time of treatment in the treating-liquid.

Unsatisfactory results are also obtained if a tow of filaments or threads is permitted to drop into and to form folds in a liquid, particularly one having a specific gravity approaching that of said tow, flowing through a static trough as tangling again results, presumably due to those portions of the folds in the centre of the trough moving faster than those nearer to the walls of the trough for, to consider any one horizontal plane of the liquid only, as is well known, the velocity of the liquid in contact with the walls of a stationary trough approaches zero while the velocity at the centre is a maximum. There are also differences in velocities, for example, between the top and the bottom of the liquid at the centre of the trough.

It has now been appreciated that as a treating liquid contained in a trough moving substantially with a velocity equal to the mean velocity of the liquid therein will be substantially free from the various velocity gradients which occur in a liquid flowing in a stationary trough it should be possible to permit a tow of filaments or threads to fall into and to form folds in a liquid con-

2

tained in such a moving trough without tangling taking place as the treated tow is removed from the liquid.

According to the present invention the method of treating a continuous tow of filaments by immersion in a treating liquid for a relatively long period of time comprises providing a horizontal ring-trough rotatable about a vertical axis, passing treating liquid in a continuous manner through said ring-trough and rotating the ring-trough with substantially the same directional speed as the mean circular velocity attained by the said treating liquid in said ring-trough, inducing a vibratory motion substantially radial to the centre of the rotating ring-trough in the tow directly above the treating liquid, permitting the thus treated tow to fall into the treating liquid and to form itself therein into folds on the floor of the rotating trough below the region immediately above the liquid from which the tow enters the liquid and also regulating the speed of rotation of the ring-trough so that on withdrawing the tow from out of the treating liquid at any desired distance away from the said region measured along the circumference of the ring-trough the said tow has remained in the treating liquid for the desired period of time.

If desired the tow can be given the said vibratory motion by passing it through a guide positioned vertically above the treating liquid and having a reciprocating movement radial to the centre of the rotating ring-trough.

It is essential in order to carry out the invention successfully that the tow undergoing treatment should be of greater density than that of the treating liquid in the rotating ring-trough. It sometimes becomes necessary therefore to give the tow a preliminary treatment before it is permitted to enter a particular treating liquid in a rotating ring-trough to make the tow of greater density than that of the treating liquid. For example, the tow may be immersed in a bath containing a particular treating liquid of a rotating ring-trough before it is allowed to enter the said treating liquid in a rotating ring-trough.

The tow of filaments or threads, if desired, can be passed from a treating-liquid contained in one rotating ring-trough into a treating-liquid contained in another rotating ring-trough in which it is again treated under conditions of continuous delay of its forward movement. The ring-troughs can be arranged independently of each other, that is to say each ring-trough is rotatable on a separate vertical axis; or the

55

ring-troughs can be arranged concentric to one another.

In one embodiment of the invention the rotatable ring-trough has a perforated base and is partly immersed in a larger and static trough which is provided with means for maintaining a constant level of liquid therein. The ring-trough is supplied continuously with treating-liquid delivered at such a rate as to make up for that which leaves it by passing through the perforations at its base. The treating-liquid is delivered from above and preferably close to the inner wall of the ring-trough. The one or more points of delivery of the treating-liquid are not connected with the ring-trough. By delivering the treating liquid in this way as for example radially from the centre of the trough any tendency towards crystallisation of the treating-liquid is lessened and the possibility of maintaining the treating-liquid at a constant predetermined high temperature throughout the treatment of the tow is increased.

In accordance with another embodiment of the invention the treating-liquid is pumped in and out of the rotating ring-trough at such a rate that the liquid is substantially static i. e. without relative motion, with respect to the rotating ring-trough. It may be desirable to provide one or more baffles between the inlet and outlet devices provided for the treating-liquid in the ring-trough.

The invention is illustrated by the following example in which parts are parts by weight except where otherwise stated and with reference to the accompanying diagrammatic drawings in which Fig. 1 is a front elevation of apparatus suitable for carrying out the method of the invention, Fig. 2 is a side elevation in direction of arrow A in Fig. 1, Fig. 3 is a plan, Fig. 4 is a section of that part of the apparatus in which the tow is treated in the first ring-trough and Fig. 5 is a section of that part of the apparatus in which the tow is treated in the second ring-trough.

#### Example

A matured caustic soda solution of groundnut globulin prepared from a solution containing 25 parts peanut globulin, 1.25 parts sodium hydroxide, 1.0 part sodium sulphite and 72.75 parts water is extruded into a coagulating bath containing 200 gm./1 sodium sulphate and 20 gm./1 sulphuric acid. The resulting tow of filaments is taken up on godets having a peripheral speed of 30 metres per minute and stretched by passing on to godets having a peripheral speed of 45 metres per minute.

The tow 1 is then led under tension to a godet 2 situated vertically above the centre line of the trough of a ring-trough 3, through a reciprocating spacing device 4 at least 3 feet above the surface of the liquor in the trough 3, and so into the trough in which the fibre is deposited in a zig-zag manner. This ring-trough 3 consists of a solid centre section 2 feet in diameter with a trough 6 inches wide and 3½ inches deep outside but integrally joined to it and is made of mild steel. This unit has a base of wire gauze 5 and revolves in a circular trough 6 3 feet 4½ inches external diameter, 1 foot 7½ inches internal diameter and 6 inches deep, also of mild steel fitted with an adjustable weir 7 so that the height of liquor in the trough may be varied at will. A solution of sodium sulphate, saturated at 15° C. is run through a pipe 8 to the centre of the centre section of the ring-trough at 15° C.

and spreads out to enter the revolving trough at a multiplicity of points. The tow sinks on to the wire gauze base 5 of the trough and is carried round with the trough which revolves once every 5 7½ minutes. Thus the time of immersion of the tow in the treating-liquid can be 7½ minutes. The tow is taken up not less than 3 inches from the fibre inlet and then stretched between two godets (9 and 10) whose peripheral speeds 10 are 35 and 52 metres per minute respectively.

After stretching, the tow passes over a godet 11 placed vertically above the centre line of the outer trough of a ring-trough consisting of two concentric troughs (12 and 13), each 6 inches 15 wide by 4 inches deep. The outside diameter of the outer trough 12 is 4 feet and the inside diameter of the inside trough 13 is 2 feet. This ring-trough is made of mild steel and is lead lined. The tow enters the outer trough 12 in a zig-zag 20 manner through a reciprocating spacing device 14 placed at least 3 feet above the liquid level in the trough. The treating liquor at 50° C., which consists of a solution of sodium sulphate saturated at 60° C. containing 1½% formaldehyde 25 at pH 5 enters the outer trough 12 through a distributing pipe 15 5½ inches long which is arranged along a diameter of the trough and at least 6 inches from the fibre inlet, and is removed by a constant level automatic syphon 16 drawing from the space between the fibre inlet 30 and outlet. The rate of rotation of the ring-trough is once in ten minutes and hence the time of immersion in the treating-liquid can be 10 minutes. The tow is picked up over a godet 17 arranged so that the fibre line coincides with a 35 diameter of the trough and that the distance between the fibre inlet and take up is at least 8 inches. The tow is stretched 50 per cent between the two godets (17 and 18) whose peripheral 40 speeds are 43 and 62 metres/minute, while the tow is immersed in a small rectangular trough 19 2 feet long, 9 inches deep, 3 inches wide. The liquor used in the trough 19 is the same as that used in the inner trough 13 and is at 90° C.

The tow enters the inner trough 13 in a zig-zag 45 manner over the godet 18 placed over the centre line of the inner trough 13 and through a reciprocating spacing device 20 at least 3 feet above the liquid level in the trough. The treating-liquor inlet 21 is by means of four pipes at right angles feeding to the inner wall of the trough 13. The treating-liquor, sodium sulphate saturated 50 at 80° C., containing 1½% formaldehyde and 20% sulphuric acid by volume, is removed by a 55 constant level automatic syphon 22 drawing from the space between the fibre inlet and take up. The temperature of the treating-liquor is 70° C. The tow is taken up over a godet 23 at least 8 inches from the inlet and washed and dried by 60 any known method.

We claim:

1. A method for treating without tangling a continuous tow of artificial wet spun protein filaments by immersion thereof in a treating liquid 65 for a relatively long period of time, said method comprising the steps of continuously flowing the treating liquid through the trough portion of a horizontally disposed, rotatable ring trough, rotating said trough in a horizontal plane about 70 its central axis at substantially the same velocity as the mean circular velocity attained by said treating liquid so that said treating liquid and trough are substantially free from velocity gradients with respect to each other, depositing 75 said tow in said ring trough radially thereof

and in a zig-zag manner, and withdrawing the thus treated tow after the desired period of treatment has elapsed.

2. The method of claim 1 wherein said artificial wet spun filaments are obtained from peanut proteins.

3. The method of claim 1 wherein said treating liquid has a greater density than said tow, the latter being given a preliminary treatment whereby its density is rendered greater than that of said treating liquid.

4. The method of claim 1 wherein said tow is successively deposited in first one ring trough and then another, said troughs being concentric to one another.

ROBIN H. K. THOMSON.  
WILLIAM E. TETLOW.  
ARCHIE M. McDONALD.

15

## REFERENCES CITED

The following references are of record in the file of this patent:

## UNITED STATES PATENTS

|    | Number    | Name                      | Date          |
|----|-----------|---------------------------|---------------|
| 5  | 2,149,708 | Von Recklinghausen et al. | Mar 7, 1939   |
| 10 | 2,251,931 | Gundelfinger              | Aug. 12, 1941 |

## FOREIGN PATENTS

|    | Number  | Country       | Date          |
|----|---------|---------------|---------------|
| 15 | 475,350 | Great Britain | Nov. 16, 1937 |